

## UNITED STATES PATENT OFFICE

2,352,579

COATING FILM FOR ZINC SURFACES AND  
METHOD OF MAKING THE SAMEJoseph J. Waters, Long Island City, N. Y., assignor  
to Etched Products Corporation, Long Island  
City, N. Y., a corporation of New YorkNo Drawing. Application November 6, 1942,  
Serial No. 464,938

3 Claims. (Cl. 106—195)

This invention relates to improvements in and methods for making coatings for metal surfaces of zinc or zinc alloys.

Up to the present time, considerable difficulty has been encountered in the coating of sheet zinc, or galvanized iron which incorporates zinc, by virtue of the apparent loss of adhesiveness of the lacquer coating upon drying. Several explanations have been offered as to the cause of this phenomenon; for example, some authorities indicate that the shrinkage of the nitro-cellulose coating, as the solvents therein become dry upon aging, causes a loss of adhesiveness of the surface of the nitro-cellulose body; others indicate that lacquers are essentially non-polar to the zinc of the metal surface, so that as the volatile solvents, which are more polar to the metal, evaporate, the now more brittle nitro-cellulose becomes even less polar and thereby further loses its adhesive properties; still others, on the one hand, attribute the break-down of coating films, in contact with zinc, to the formation of occluded oxygen which, on coming to the surface of the metal at the film layer, undermines the coating film and destroys its adhesion, while, on the other hand, others theorize to the effect that there is a decomposition of the nitro-cellulose in which free acid, liberated therefrom, reacts with the zinc surfaces, with the zinc acting as a catalyst, with the result that a progressive electrolytic action reduces the polarity and the adhesion of the nitro-cellulose to the zinc surface.

Various mechanical expedients, such as tumbling or blasting; chemical expedients, such as etching or coating with various organic salts; and, lastly, special priming coats, incorporating resins or the like, have been attempted, but the problem has remained unsolved.

It has been suggested in the literature, that priming coats, incorporating zinc dust and resinous materials, might eliminate the present difficulties, but this procedure has two inherent weaknesses: first, the zinc dust will discolor the primer and the succeeding lacquer coatings; and, secondly, the use of a primer, followed by a further outside coating, introduces an undesired double thickness of coatings and the expense in both time and material of two coating operations, particularly in the manufacture of etched indicia plates, or the like, where it is essential not only that a single lacquer layer or coating be applied, but that such coating be very thin.

In contradistinction to some of the theories advanced in the literature, it is my belief that it is not a matter of the drying of nitro-cellulose

solvents which controls adhesion of a lacquer to a zinc surface, but rather that the lacquer, by virtue of the absence of a metallic salt, is ab initio and always remains substantially non-polar to a zinc surface and on this basis, with the desire to increase the polarity of the lacquer to zinc, I have treated the lacquer, before application, as follows:

I have added to a lacquer of any color a relatively small amount of zinc dust of relatively fine mesh and permitted the zinc dust to stand for a short period of time; whereupon the zinc dust substantially entirely settled out. Thereafter, I decanted the lacquer solution from the settled zinc dust residue. The decanted lacquer, when applied as the only coating to the zinc surface, has been found to firmly adhere, even after aging of several months. My preferred preparations comprise one ounce of zinc dust of 300 mesh and finer to a gallon of nitro-cellulose lacquer, and the settling out of the zinc dust commences immediately and, at the end of twelve (12) hours, has settled out in an amount of more than ninety-nine (99%) per cent, after which period, the thus treated lacquer is decanted.

As above stated, I have found that substantially all of the zinc dust applied to the lacquer settles out as a residue, and consider that essentially one of three phenomena occurs: (a) a zinc salt is formed with some of the acid in the lacquer, thereby rendering the same more polar to the zinc by virtue of the presence of the zinc salt; or (b) the zinc dust reduces some of the constituents of the lacquer, which are oxidizers, or have a tendency to liberate oxygen upon aging; or (c) the zinc dust possibly serves as an absorptive medium for that constituent of the lacquer which normally initially or progressively renders the nitro-cellulose lacquer non-polar to the zinc surface being coated.

In any case, I do not consider that I have ascertained the actual chemical, physical or electrochemical phenomenon that occurs by virtue of my treatment of the nitro-cellulose lacquer with the zinc dust as above defined, other than to have discovered that such treatment renders the nitro-cellulose firmly adhesive as a coating to a zinc surface.

Various changes and modifications may be made to the details of the invention without departing from the broader spirit and scope thereof, as set forth in the following claims:

I claim:

1. A method for treating a pyroxylin lacquer to render the same adhesive to zinc surfaces,

which comprises adding zinc dust to the lacquer and, after permitting the zinc dust to settle, decanting therefrom the thus treated pyroxylin lacquer.

2. A coating for and rendered adhesive to zinc metal surfaces comprising the decanted portion of an intermixture of pyroxylin lacquer and zinc dust from which the zinc dust has settled out.

3. A method of rendering pyroxylin lacquer more adhesive to zinc surfaces for forming a coating therefor which comprises intermixing zinc dust with pyroxylin lacquer, permitting the zinc dust to settle out and separating the thus treated pyroxylin lacquer from the settled-out zinc dust.

JOSEPH J. WATERS.